



US006120914A

# United States Patent [19]

Troughton et al.

[11] Patent Number: 6,120,914

[45] Date of Patent: Sep. 19, 2000

[54] HOG FUEL BOARD

[75] Inventors: **Gary Ellis Troughton; Ken Lui Chan; Kenneth Gordon Love**, all of Vancouver, Canada

[73] Assignee: **Forintek Canada Corp.**, Canada

[21] Appl. No.: **08/988,914**

[22] Filed: **Dec. 11, 1997**

532991 11/1956 Canada .  
90-03527 5/1990 Rep. of Korea .

Primary Examiner—Bruce H. Hess

Assistant Examiner—Michael Grendzynski

Attorney, Agent, or Firm—Oppenheimer Wolff & Donnelly LLP

## [57] ABSTRACT

A hog fuel board is made by placing a hog fuel matrix with flexible non-sticking layers on outside surfaces between screens in a preheated platen press and pressing the matrix to preset stops and for a predetermined time and pressure to cause adhesives naturally present in the hog fuel to disperse throughout the board. The process requires heating platens higher than used for particle board but avoids using a vacuum press. There is also supplied a hog fuel veneer board with a hog fuel matrix sandwiched between veneer sheets and a lumber product with a hog fuel coating thereon.

## [56] References Cited

### FOREIGN PATENT DOCUMENTS

8775037 1/1988 Australia .

17 Claims, 1 Drawing Sheet





FIG. 1



FIG. 2



FIG. 3



FIG. 4

**HOG FUEL BOARD**

This application is a divisional application of U.S. patent application Ser. No. 08/672,321, now U.S. Pat. No. 5,725,818 entitled MANUFACTURE OF HOG FUEL BOARD (as amended), filed Jun. 28, 1996, by Gary Ellis Troughton, Ken Lui Chan, and Kenneth Gordon Love.

**TECHNICAL FIELD**

The present invention relates to a composite wood board product and more specifically a board product formed with a hog fuel matrix therein utilizing adhesives naturally present in the hog fuel that are dispersed throughout the board product during formation.

**BACKGROUND ART**

Hog fuel is generally sawmill refuse that has been fed through a disintegrator or hog by which the various sizes and forms are reduced to a practically uniform size of chips or shreds. Hog fuels generally contain approximately 70% to 95% bark with the residue being primarily wood.

Bark boards made without synthetic resins are known. In an Article entitled "Bark Boards Without Synthetic Resins" published by S. Chow in Volume 25, No. 11, of the Forest Products Journal, pages 32 to 37, dated November, 1975, is disclosed making bark boards without the addition of synthetic resin by forming a bark matrix into a mat and then compressing the mat in a platen press at a predetermined pressure and temperature. During the pressing step a vacuum is applied continuously to the platens to withdraw steam and water vapour. The boards were tested for dry bending strength and compared with particle board. Favourable results were obtained, however, the product has never achieved success in the marketplace.

It has now been found that by utilizing hog fuel rather than carefully selected bark, one includes at least a small percentage of wood with the bark and a percentage of wood over 5% adds additional strength to a bark board product. Inasmuch as hog fuel already has wood particles therein, it is not necessary to separate the wood particles from the bark but use the hog fuel as it comes from the hogging process to remove the bark. Furthermore, it has now been found that one can produce a hog fuel board without having to apply a vacuum to a platen press. The vacuum step is an expensive operation which may well have prevented the bark boards disclosed by Chow from being commercially feasible.

In the past hog fuel was burned, however, in today's environmental conscious environment, burning is not appropriate and therefore hog fuel accumulates in sawmills. Thus, a competitive product utilizing hog fuel provides use of what is now a waste product and solves a disposal problem.

**DISCLOSURE OF INVENTION**

The hog fuel board of the present invention is manufactured in existing equipment modified to have higher platen temperatures, has strength comparable with particle board and does not require the use of added adhesives but utilizes adhesives naturally present within the hog fuel. Boards made of hog fuel have greater strength in bending than boards made of bark alone. Furthermore, hog fuel boards have excellent dimensional stability for all uses as compared to other wood composite board products.

In one embodiment, the present invention provides a hog fuel veneer board comprising hog fuel matrix containing about 80% bark, the remainder being primarily wood

residues, sandwiched between veneer sheets, the board having only adhesives naturally present in the hog fuel to maintain board cohesion, the adhesives dispersed throughout the matrix from heat and pressure applied to form the board. The veneer sheets provide smooth woodgrain exterior surfaces suitable for furniture and many other uses.

The present invention also provides a method of forming a hog fuel board comprising the steps of placing a hog fuel matrix containing between about 70% and 95% bark, the remainder being primarily wood residues, with flexible non-sticking layers on outside surfaces, between screens in a preheated platen press and pressing the matrix in the platen press to preset stops for a predetermined time and at a predetermined pressure to cause adhesives naturally present in the hog fuel to disperse throughout the board.

In another embodiment, a hog fuel coated board has hog fuel matrix containing about 80% bark, the remainder being primarily wood residues, on one or both sides of a lumber product. The finished board has the natural protection that bark gives to a tree, and provides improved chemical resistance, fire resistance and decay resistance over standard untreated lumber products.

**BRIEF DESCRIPTION OF DRAWINGS**

In drawings which illustrate embodiments of the invention,

FIG. 1 is a sectional view showing a hog fuel board in a platen press,

FIG. 2 is a sectional view showing a hog fuel coating on a lumber board in a platen press,

FIG. 3 is a sectional view showing a lumber product with hog fuel coatings on both sides,

FIG. 4 is a sectional view showing a hog fuel veneer board in a platen press.

**MODES FOR CARRYING OUT THE INVENTION**

The preparation of a hog fuel board is a one step process. Hog fuel, which has approximately 70% to 95% bark, the remainder being wood residues, is dried to about 3% to 5% moisture content and then ground in a Wiley mill or suitable grinder to pass a 5 mesh screen. Thus, the hog fuel has approximately a 4mm size particles. The preferred hog fuel consistency is about 80% bark, this provides improved bending strength. If the wood content exceeds about 30% then there may be insufficient natural adhesives present to bond the board together.

As shown in FIG. 1, a hog fuel matrix 10 is laid between two impermeable tetrafluoroethylene polymer sheets 12, generally known under the trademark TEFLON. These sheets represent flexible non-sticking layers to prevent the hog fuel sticking. This preform assembly is placed between interwoven stainless steel wire mesh screens 14 in a pre-heated platen press 16. The combination of the non-sticking layers 12 and the screens 14 permit the gases produced in the heating and pressing stage to expand against the screens 14 and produce small channels or grooves allowing the gases to escape. If solid platens are used without screens then the gases remain trapped in the board, and delamination occurs.

The platen press 16 is preheated to a preset temperature higher than used for the normal production of particle board, and the preform assembly is compressed at a predetermined pressure to stops which determine board thickness. Pressure is maintained on the board in the press 16 for a preset time to permit the natural adhesives in the hog fuel to disperse

throughout the matrix **10** and act as an adhesive to hold the board together.

The resulting hog fuel board has excellent dimensional stability. The bark provides a natural protection against decay, improved chemical resistance over other wood products and better flame resistance properties.

In another embodiment, a hog fuel coating is applied to one or both sides of a lumber product such as a board. FIG. 2 shows a single side coating wherein a hog fuel matrix **10** is placed on a non-sticking layer **12** and a lumber **20** is placed between the screen mesh **14** and the matrix **10**. In FIG. 3, two sides of the lumber **20** are coated, therefore hog fuel matrix **10** is placed on both sides. No additional adhesive is required and the natural adhesives in the hog fuel joins the hog fuel particles to the lumber **20**.

In one example, 200 grams of hog fuel at 5% moisture content was placed on a 13"×13" surface on both sides of a board. The assembly was pressed to stops. Thus the density of the coating is determined by the placing of the stops and the quantity of hog fuel used. The densified bark surface produced was  $\frac{1}{16}$ ".

As shown in FIG. 4, a hog fuel matrix **10** is sandwiched between thin veneer sheets **22**. The thickness of hog fuel is dependent upon the requirements of the board and in some cases is ruled by the space available in the platen press. Impermeable tetrafluoroethylene polymer sheets **12** are placed on both sides of the veneer sheets **22** to prevent sticking in the press. This complete preform assembly is then placed between screens **14** in a preheated platen press **16**. In a preferred embodiment the preheated platen press **16** is preheated to a temperature of about 300° C. or 260° C. and the assembly is compressed to stops, representing a preset thickness of board, and maintained at a pressure to permit the natural adhesives within the hog fuel to disperse throughout the matrix **10** and act as an adhesive to join the hog fuel particles to the veneer sheets **12**.

In one embodiment the tetrafluoroethylene polymer sheets are  $\frac{1}{64}$ " thick and are incised to ensure that any gas present within the matrix can escape from the preform assembly and the screens permit gases to pass to the sides of the press.

No vacuum is required for the pressing step, thus expensive vacuum platen presses are not needed.

In a preferred embodiment the preform assembly of the hog fuel veneer board is placed between screens and positioned in a preheated platen press at 260° C., the assembly is compressed to stops with an initial pressure of 400 psi for one minute and then the pressure is reduced to 175 psi for nineteen minutes.

In another embodiment the press is heated to 300° C., the preform assembly is compressed to stops with an initial pressure of 400 psi for one minute and then the pressure is reduced to 175 psi for four minutes. This latter pressing condition is more practical for commercial operation.

In one example a hog fuel matrix composed of 900 grams of hog fuel powder (approximately 4 mm size particles), about 80% bark, the remainder being wood residues, having a moisture content average of 30%, was placed in an open ended 12"×12" box, 5" deep between  $\frac{1}{16}$ " thick 13×13" birch veneer sheets which had been incised, and then placed between thin 15"×15" tetrafluoroethylene polymer sheets. The tetrafluoroethylene polymer sheets were placed on a 15"×15" interwoven stainless steel wire mesh screen (2 mm thick). A slight pressure (about 10 psi) was exerted in the press while the box was removed. The tetrafluoroethylene polymer sheet and the screen were then placed on top of the

assembly and it was pressed to stops at the pressure and temperature described. The bond thickness was approximately 0.4 inches thick. A 13"×13" board was produced and it was found that the board has a natural resistance to decay as the bark is the strongest and most protective portion of a tree, therefore all the protective properties of bark are applied to the wood product. In another test, a  $\frac{1}{32}$ " permeable pine veneer was used which was not incised. The veneers have to permit moisture to escape onto the screens. 10 Hog fuel board can be formed using both a hardwood veneer such as birch, and a softwood veneer such as pine. Other wood species can also be used.

In yet another embodiment a non-sticking reagent was sprayed onto the outside veneer sheets to act as a flexible non-sticking layer in place of the tetrafluoroethylene polymer sheets.

Bending data for pure bark and hog fuel boards are shown in Table 1. An improvement in MOR and MOE occurs which is due to the addition of wood in the hog fuel.

TABLE 1

| Bending Data for Pure Bark and Hog Fuel Boards* |                           |                          |                |                  |                  |
|-------------------------------------------------|---------------------------|--------------------------|----------------|------------------|------------------|
|                                                 | Species and type of board | Board thickness (inches) | Density (g/cc) | Avg.** MOR (psi) | Avg.** MOE (psi) |
| 25                                              | Pine bark (pure)          | 0.19                     | 0.67           | 175              | 33,500           |
| 30                                              | Pine hog fuel             | 0.19                     | 0.68           | 775              | 152,000          |
| 35                                              | Spruce bark (pure)        | 0.19                     | 0.70           | 536              | 89,000           |
| 40                                              | Spruce hog fuel           | 0.19                     | 0.69           | 940              | 174,000          |

\*boards pressed 300° C. for 5 mins

\*\*average of 2 bending samples

35 The durability properties of the spruce hog fuel veneer boards are reflected by the high retention of MOR (79%) and MOE (75%) after a 2-hour boil test as shown in Table 2. As well the dimensional stability was good because the hog fuel veneer boards should average 7.5% swelling after the 2-hour boil test.

TABLE 2

| Bending data for spruce hog fuel veneer boards* |                                     |                            |                  |                  |                  |                |
|-------------------------------------------------|-------------------------------------|----------------------------|------------------|------------------|------------------|----------------|
|                                                 | Veneer Overlay                      | Board Thickness** (inches) | Density** (g/cc) | Avg. MOR** (psi) | Avg. MOE** (psi) | Test Condition |
| 45                                              | 0.031-inch incised birch veneer     | 0.24                       | 0.75             | 4500             | 810,000          | Dry            |
| 50                                              | 0.031-inch non-incised birch veneer | 0.24                       | 0.74             | 4225             | 775,000          | Dry            |
| 55                                              | 0.062-inch non-incised birch veneer | 0.43                       | 0.80             | 7000             | 1,270,000        | Dry            |
|                                                 |                                     |                            |                  | 5500             | 950,000***       | Boil           |
|                                                 | 0.031-inch non-incised pine veneer  | 0.43                       | 0.73             | 3170             | 736,000          | Dry            |

\*boards pressed at 260° C. for 20 min.

\*\*average of 2 bending samples

\*\*\*boil test - bending samples were tested after a 2-hour boil test

65 The percentage thickness swell of pine hog fuel boards is shown in Table 3 and spruce hog fuel boards in Table 4. As can be seen after a 2-hour boil test, the boards exhibited excellent dimensional stability properties that indicate they could be used in exposed or semi-exposed situations.

TABLE 3

| % Thickness swelling for pine hog fuel boards<br>(2-hour boil test) |                   |            |
|---------------------------------------------------------------------|-------------------|------------|
| Sample                                                              | Density<br>(g/cc) | % Swelling |
| 1                                                                   | 0.85              | 7.5        |
| 2                                                                   | 0.82              | 5.9        |
| 3                                                                   | 0.82              | 6.0        |
| 4                                                                   | 0.75              | 5.9        |
| 5                                                                   | 0.83              | 6.6        |
| Avg                                                                 | 0.81              | Avg<br>6.4 |

TABLE 4

| % Thickness swelling for spruce hog fuel boards<br>(2-hour boil test) |                   |             |
|-----------------------------------------------------------------------|-------------------|-------------|
| Sample                                                                | Density<br>(g/cc) | % Swelling  |
| 1                                                                     | 0.94              | 6.0         |
| 2                                                                     | 0.87              | 6.1         |
| 3                                                                     | 0.86              | 7.1         |
| 4                                                                     | 0.82              | 8.4         |
| 5                                                                     | 0.85              | 5.7         |
| Avg                                                                   | 0.87              | Avg<br>6.7% |

The tests for MOR and MOE were done according to CSA 3-0188.1-M-78 standard (Interior mat formed wood particle board). The range of requirements in this standard is 1,300 to 2,400 psi for minimum modulus of rupture (MOR), 160,000 to 360,000 psi for minimum modulus of elasticity (MOE) and 40 to 65 psi for minimum internal bond (IB).

Some examples of board strengths for spruce and pine hog fuel boards are shown in Tables 5 and 6 respectively. The average internal bond strengths are much higher than the standards for the highest grade particle board.

TABLE 5

| Internal bond strength data for spruce hog fuel boards |                   |                        |
|--------------------------------------------------------|-------------------|------------------------|
| Sample                                                 | Density<br>(g/cc) | Internal Bond<br>(psi) |
| 1                                                      | 0.82              | 112.1                  |
| 2                                                      | 0.91              | 144.4                  |
| 3                                                      | 0.85              | 163.3                  |
| 4                                                      | 0.83              | 111.1                  |
| 5                                                      | 0.92              | 140.0                  |
| 6                                                      | 0.83              | 94.9                   |
| 7                                                      | 0.92              | 129.3                  |
| 8                                                      | 0.85              | 130.0                  |
| 9                                                      | 85                | 120.7                  |
| 10                                                     | 0.79              | 109.0                  |
|                                                        | 0.86              | Avg<br>125.5           |

TABLE 6

| Internal bond strength data for pine hog fuel boards |                   |                        |
|------------------------------------------------------|-------------------|------------------------|
| Sample                                               | Density<br>(g/cc) | Internal Bond<br>(psi) |
| 1                                                    | 0.84              | 94.3                   |
| 2                                                    | 0.84              | 75.6                   |
| 3                                                    | 0.87              | 106.3                  |
| 4                                                    | 0.85              | 67.6                   |
| 5                                                    | 0.87              | 73.9                   |

TABLE 6-continued

| Internal bond strength data for pine hog fuel boards |                   |                        |
|------------------------------------------------------|-------------------|------------------------|
| Sample                                               | Density<br>(g/cc) | Internal Bond<br>(psi) |
| 6                                                    | 0.87              | 74.9                   |
| 7                                                    | 0.84              | 86.5                   |
| 8                                                    | 0.90              | 78.1                   |
| 9                                                    | 0.88              | 80.6                   |
| 10                                                   | 0.88              | 92.6                   |
| Avg                                                  | 0.86              | Avg<br>83.0            |

The hog fuel boards and board coatings are formed in a single step without having to have overlays added. The end product was found to have strength properties consistent with particle board and which had a natural resistance to decay. The bark tends to be more resistant to chemicals than plain wood as it is a protective coating for the tree.

Various changes may be made to the embodiments shown herein without departing from the scope of the present invention which is limited only by the following claims.

What is claimed is:

1. A hog fuel board comprising a compressed hog fuel matrix, the matrix containing about 70% to about 95% of a bark by weight, the remainder of the matrix being primarily wood residues, the board having only adhesives naturally present in the hog fuel to maintain board cohesion, the adhesives being dispersed throughout the matrix from a heat and a pressure applied to form the board, the board having a modulus of rupture (MOR), modulus of elasticity (MOE) or dimensional stability greater than a bark board, obtainable by applying the heat and the pressure to the bark alone.
2. The hog fuel board of claim 1 wherein the MOR of the board is greater than about 600psi.
3. The hog fuel board of claim 1 wherein the MOR of the board is greater than about 700psi.
4. The hog fuel board of claim 1 wherein the MOE of the board is greater than about 90,000psi.
5. The hog fuel board of claim 1 wherein the MOE of the board is greater than about 100,000psi.
6. The hog fuel board of claim 1 wherein the MOE of the board is greater than about 150,000psi.
7. The hog fuel board of claim 1 wherein the dimensional stability of the board is such that the board survives a 2-hour boil test.

8. The hog fuel board of claim 1 wherein the dimensional stability of the board is such that the board has an edge thickness swelling of less than about 10% in a 2-hour boil test.
9. The hog fuel board of claim 1 wherein the matrix contains about 75 % to about 90% of the bark by weight.
10. The hog fuel board of claim 1 wherein the matrix contains about 80% of the bark by weight.
11. A hog fuel veneer board comprising: a compressed hog fuel matrix sandwiched between veneer sheets the hog fuel matrix containing about 70% to 90% bark by weight, the remainder of the matrix being primarily wood residues, the board having only adhesives naturally present in the hog fuel to maintain board cohesion, the adhesives dispersed throughout the matrix from heat and pressure applied to form the board.

12. The hog fuel veneer board according to claim 11 wherein the veneer sheets are incised.
13. The hog fuel veneer board according to claim 12 wherein the veneer sheets are birch having a thickness of  $\frac{1}{16}$ ".

**14.** The hog fuel veneer board according to claim **11** wherein the veneer sheets are pine having a thickness of  $\frac{1}{32}$ ".

**15.** A lumber product with a hog fuel coating thereon comprising:

a compressed hog fuel matrix coating containing about

70% to 90% bark by weight, the remainder being primarily wood residues, the matrix coating held together and held to the lumber product only by adhesives naturally present in the hog fuel, to maintain

cohesion in the matrix and to the lumber product, the adhesives dispersed throughout the matrix from heat and pressure applied to apply the coating to the lumber product.

**16.** The lumber product according to claim **15** wherein hog fuel coating is on both sides of the lumber product.

**17.** The lumber product according to claim **15** wherein the hog fuel coating is approximately  $\frac{1}{16}$ " thick.

\* \* \* \* \*